

## 1

2,698,842

## FIBERS OF ACRYLONITRILE-ALKYL ALPHA-ACYLAMINO ACRYLATE COPOLYMER

Joseph B. Dickey, Rochester, N. Y., Harry W. Coover, Kingsport, Tenn., and Theodore E. Stainin, Rochester, N. Y., assignors to Eastman Kodak Company, Rochester, N. Y., a corporation of New Jersey

No Drawing. Application August 17, 1950,  
Serial No. 180,104

3 Claims. (Cl. 260—85.5)

This invention relates to spinning copolymers derived from acrylonitrile and alkyl esters of  $\alpha$ -acetamino acrylic acid in order to form filaments or like shaped articles therefrom. More particularly, this invention concerns an improved process for spinning such acrylonitrile copolymers whereby shaped articles such as filaments, fibers and the like are produced substantially free of voids, having an attractive lustrous appearance, a high tenacity, an improved light and gas fastness, an improved dyeability and moisture affinity and, in addition, having the important characteristic of a relatively high temperature softening point.

The production of yarn from unmodified polyacrylonitrile has been achieved heretofore and such yarn has a high tenacity with a desirable high softening point of about 220° C. These properties, particularly the high softening point, which is lacking in other vinyl polymer fibers, is a necessary characteristic if the fiber is to be employed in textile materials. Such unmodified polyacrylonitrile yarns, however, lack other properties which are necessary in a generally useful textile material suitable for clothing manufacture. These properties, which are not found in unmodified polyacrylonitrile yarns or textiles, are good dyeability and affinity for moisture. Without these additional properties the usefulness of the yarn is limited for many purposes.

The dye affinity and moisture absorption of polyacrylonitrile type yarn has been improved by copolymerizing acrylonitrile with compounds containing hydrophylic groups; e. g., carboxyl, ester, amido, amino and hydroxyl groups. This may readily be accomplished by employing as the other polymer such compounds such as vinyl acetate, acrylamide and acrylic acid. Desirable improvements as respects dyeability and moisture absorption are secured by polymerizing with about 15-40% of these modifiers but at the expense of the softening point of the fiber. The inclusion of such modifiers invariably results in a lowering of the softening point of from 40-100° C. depending on the nature and amount of modifier present. Such modified polyacrylonitrile fibers shrink greatly in hot water and fuse under a flat-iron at normal ironing temperatures which are employed for pressing textile fabrics. Consequently, the polyacrylonitrile fibers thus modified are still of limited application in the textile industry.

An object, therefore, of the present invention is an improved process for forming copolymers of acrylonitrile and alkyl esters of  $\alpha$ -acylamino acrylic acid into shaped articles.

Another object of the invention is to provide new and improved filaments and yarns from copolymers of acrylonitrile and alkyl esters of  $\alpha$ -acyl amino acrylic acid characterized by freedom from voids, a lustrous appearance, a high tenacity and extensibility, an improved dyeability, an improved light and gas fastness, and a relatively high sticking temperature.

Still another object is to provide a process for wet spinning copolymers of acrylonitrile and an alkyl  $\alpha$ -acylamino acrylate into filaments in an aqueous coagulating bath.

Yet another object is a process of spinning such acrylonitrile modified polymers which includes stretching the filaments to improve their structure.

## 2

Other objects will be apparent from the following detailed description of the invention.

In accordance with the invention, we have found that solutions of copolymers of acrylonitrile and alkyl esters of  $\alpha$ -acylamino acrylic acid containing 15 to 40% of the ester by weight may be forced through a suitable spinnerette and coagulated in an aqueous bath to form a filament which preferably is then passed through an atmosphere of hot air maintained approximately from 60° C. to 140° C. The filament is preferably stretched while passing through the hot air atmosphere in accordance with the amount of draft desired. Stretching improves the continuity of the filament and reduces voids therein. Bundles of such filaments may be twisted into thread by any desirable method. Yarns which contain acrylonitrile copolymerized with 20-35% of the ester especially have excellent affinity for acetate, basic, acid and insoluble vat dyes and good affinity for direct and soluble vat dyes. Of special importance is their relatively high sticking temperatures, fastness to light and gas fumes, and desirable moisture affinity. We have found that certain blue dyes which are not fast to gas fumes when on acetate yarn are substantially unaffected when the fibers of the instant invention are dyed with them. Any suitable spinning apparatus known in the prior art and equipped with means for forcing the spinning solution through a spinnerette into a coagulating bath may be employed. The associated drying chamber may be conventional and the stretching may be carried out by a system of drums running at increasing rates as is common in this art.

The alkyl  $\alpha$ -acylaminoacrylates which may be employed in our invention to copolymerize with acrylonitrile may be represented by the following general formula:

35



40 wherein R represents an alkyl group such as methyl, ethyl, n-propyl, isopropyl, n-butyl, isobutyl, etc., groups (e. g., an alkyl group containing from 1 to 4 carbon atoms), and R<sub>1</sub> represents an alkyl group such as methyl, ethyl, n-propyl, isopropyl, etc., groups (e. g., an alkyl group containing from 1 to 3 atoms).

45 Representative esters, in accordance with the above general formula, for example, include: Methyl  $\alpha$ -acetaminoacrylate, ethyl  $\alpha$ -acetaminoacrylate, n-propyl  $\alpha$ -acetaminoacrylate, isopropyl  $\alpha$ -acetaminoacrylate, n-butyl  $\alpha$ -acetaminoacrylate, methyl  $\alpha$ -propionaminoacrylate, ethyl  $\alpha$ -propionaminoacrylate, n-butyl  $\alpha$ -propionaminoacrylate, methyl  $\alpha$ -n-butyraminoacrylate, ethyl  $\alpha$ -n-butyraminoacrylate, isobutyl  $\alpha$ -n-butyraminoacrylate, methyl  $\alpha$ -isobutyraminoacrylate, ethyl  $\alpha$ -isobutyraminoacrylate, n-propyl  $\alpha$ -isobutyraminoacrylate, iso-butyl  $\alpha$ -isobutyraminoacrylate.

50 The alkyl  $\alpha$ -acylaminoacrylates represented by the above general formula can be prepared according to the general method described in the copending application, Serial No. 87,356 filed April 13, 1949, of H. W. Coover, Jr., and Joseph B. Dickey, now Patent No. 2,548,518. The process described in that application comprises reacting an alkali metal salt of an  $\alpha$ -acylaminoacrylic acid with a dialkyl sulfate. The alkali metals useful for this

55 purpose comprise those set forth in Serial No. 87,356 and also those alkali metal salts of the  $\alpha$ -acylaminoacrylic acids described in the copending application, Serial No. 132,216, filed December 9, 1949, of H. W. Coover, Jr., and Joseph B. Dickey, now Patent No. 2,622,074. Suitable methods for preparing copolymers of acrylonitrile and alkyl  $\alpha$ -acylaminoacrylates are described in the patent literature and methods particularly suitable for producing the copolymers advantageously employed in accordance with our invention are described in the examples included hereinafter.

70 75 To prepare the spinning solutions the copolymers of

acrylonitrile and alkyl  $\alpha$ -acylamino acrylate may be dissolved in various solvents for example dimethyl formamide, dimethylacetamide, ethylene carbonate, ethylene carbamate, N - methyl - 2 - pyrrolidone,  $\gamma$ -butyrolactone, succinonitrile,  $\gamma$ -valerolactone, and tetramethylene cyclic sulfone.

The invention is further illustrated in the following examples:

*Example 1.*—Two parts of ethyl  $\alpha$ -acetamino acrylate and 8 parts of acrylonitrile are added to 100 parts of distilled water to which 0.1 part of ammonia persulfate and 0.2 part of sodium bisulfate are added. The reaction vessel is sealed from the outside air and maintained at 35-40° C. for 18 hours. A fine white insoluble polymer is formed which is filtered off and thoroughly washed with water, then dried. 9.1 parts of a copolymer of acrylonitrile and ethyl  $\alpha$ -acetamino acrylate are obtained which softens at 200° C. on a Dennis bar and which contains 23.3% of ethyl  $\alpha$ -acetamino acrylate as calculated from carbon analysis. This copolymer is readily soluble in dimethyl formamide and dimethyl acetamide. The inherent viscosity is 2.1 measured as a 0.25% solution in dimethyl formamide.

*Example 2.*—Three parts methyl  $\alpha$ -acetamino acrylate and 7 parts acrylonitrile are added to 100 parts of distilled water to which 0.1 part of ammonia persulfate and 0.2 part of sodium bisulfate are added. The reaction vessel is sealed from the outside air and maintained at 35-40° C. for 18 hours. A fine white insoluble polymer is formed which is filtered off and thoroughly washed with water, then dried. 7.5 parts of copolymer of acrylonitrile and methyl  $\alpha$ -acetamino acrylate containing 27.2% of methyl  $\alpha$ -acetamino acrylate are obtained which had softening point of 220° C. as measured by a Dennis bar. The inherent viscosity is 1.9 as measured in a 0.25% solution in dimethyl formamide.

*Example 3.*—A spinning procedure by which these copolymers may be spun into filaments, in accordance with another feature of the invention, is now described.

A spinning solution of the copolymer prepared in Example 2 was made up by dissolving 6.4 grams of polymer in 40 cc. of dimethyl formamide. This dope was filtered by pressure into a spinning chamber containing a 0.1 mm. single hole spinnerette. The dope was extruded into a water bath by applying 40 p. s. i. pressure from a nitrogen tank. The coagulated monofilament was taken up on a roll rotating at a peripheral rate of 18 ft./min., then drawn through a hot-air chamber at 140° C. and wound on a drum traveling at a peripheral rate of 72 ft./min. This stretching rate is regulated according to the amount of draft desired and can be increased up to 126 ft./min. The thread guide through which the filament passes just before being wound on the drum is attached to a mechanism which can shift its position every fifty revolutions of the drum so that individual bundles of fifty monofilaments can be collected from the drum and twisted into a thread which can be tested on conventional textile yarn testing machinery. The yarn samples were tested before and after shrinkage in boiling water.

The fibers containing 20-35% of the ester had excellent affinity for acetate, basic, acid and insoluble vat dyes and good affinity for direct and soluble vat dyes.

*Example 4.*—Similar acrylonitrile copolymers were prepared containing 15 to 40% of an alkyl  $\alpha$ -acylamino-acrylate and spun in accordance with the methods described above and other desirable properties of fibers made in accordance with the present invention are shown in the following tables.

Table II

The effect of the composition of the copolymer on the sticking point of the fibers as measured on a Dennis bar is illustrated in the following table:

|    | Percent Methyl ester | Sticking Point, °C. | Percent Ethyl ester | Sticking Point, °C. |
|----|----------------------|---------------------|---------------------|---------------------|
| 10 | 15.....              | 215                 | 23.....             | 200                 |
|    | 22.....              | 210                 | 25.....             | 185                 |
|    | 27.....              | 185                 | 33.....             | 185                 |
|    | 32.....              | 185                 |                     |                     |
| 15 | 40.....              | 190                 |                     |                     |

The general effect of increasing the amount of alkyl  $\alpha$ -acylamino acrylate above 40% is to further lower the softening point of the copolymer and no very significant improvement in dyeing properties is gained. However, if the percentage of the alkyl  $\alpha$ -acylamino acrylate in the acrylonitrile copolymer is reduced below 15% other undesirable features are introduced. For example, the composition of copolymer of 5% methyl  $\alpha$ -acetamino acrylate and 95% acrylonitrile disclosed in U. S. Patent 2,461,383 of February 8, 1949 is only very slightly better as respects dye affinity and moisture absorption than unmodified polyacrylonitrile and consequently is not satisfactory as a composition to make into textile fabrics. The practical range of composition of these copolymers lies between 15 and 40% and the most desirable properties are obtained at 20-35%.

The polyacrylonitrile useful in practicing our invention can be prepared according to the process described in U. S. Patent 2,434,054 of January 6, 1948, or U. S. Patent 2,296,403 of September 22, 1942. Other processes which can be employed for preparing polyacrylonitrile are described in copending applications, Serial Nos. 49,651, 49,652, 49,653, all filed September 16, 1948, in the name of T. E. Stanin, H. W. Coover, Jr., and J. B. Dickey, the first two of which issued respectively as Patent Nos. 2,629,711 and 2,629,712 and the third is now abandoned.

As indicated in the foregoing examples, a coagulating bath of distilled water may be advantageously employed in our wet spinning process. However, if desired the bath may also contain some of the solvent corresponding to the solvent employed in preparing the spinning solution that is being spun. We have found that the precipitating bath may be comprised of water varying from 25 to 100%, the balance being a solvent of the type contained in the dope or another solvent for the copolymer. While there is no need of incorporating special salts or alcohols into the bath when operating in accordance with the present invention, it is apparent that the incorporation of small amounts of some of these salts and chemicals are not injurious.

The filaments should generally remain in the aqueous bath for a sufficient time and distance to substantially or nearly completely coagulate the filaments. The subsequent high temperature drying step is an important feature of this process. The temperature of the air for drying purposes must be at least 60° C. and may be as high as 140° C., preferably 80° C. to 110° C. It is also desirable that the filament contain an appreciable quantity of solvent when it enters the drying chamber, usually 5 to 25% of the solvent associated with the polymer in the spinning solution. The high temperature of the drying permits rapid removal of the water and most of the residual solvent and at the same time the presence of the solvent permits the polymer to flow

Table I

| Polymer Composition   | Unshrunken |               | Shrinkage in Water at 100° | Shrunken |      | Elastic Recovery | Moisture Abs. 65% rel. hum. |
|-----------------------|------------|---------------|----------------------------|----------|------|------------------|-----------------------------|
|                       | Tenacity   | Extensibility |                            | Ten.     | Ext. |                  |                             |
| 22% methyl ester..... | 2.56       | Percent       | Percent                    | 11       | 2.0  | Percent          | Percent 4.1                 |
| 27% methyl ester..... | 1.46       | 12            | 17                         | 1.45     | 20   | 67               |                             |
| 32% methyl ester..... | 1.48       | 12            | 19                         | 1.57     | 23   | 68               | 4.8                         |
| 40% methyl ester..... | 1.63       | 8             | 16                         | 1.27     | 19   | 69               |                             |
| 23% ethyl ester.....  | 1.40       | 13            | 12                         | 1.46     | 20   | 69               | 3.6                         |
| 33% ethyl ester.....  | 1.62       | 10            | 13                         | 1.74     | 20   | 70               | 5.9                         |

slightly, thus removing voids in the yarns produced in the spinning bath. Under proper conditions, the yarn emerges from the drying operation without any appreciable number of voids, and is dry enough to permit stretching to produce greater strength. The heating step is preferably employed, since these freshly spun yarns, if dried at temperatures appreciably less than 60° C., say from 25° C. to 50° C., can be stretched only with difficulty and will contain numerous voids and be generally unsuited for use in the textile art.

We claim:

1. A synthetic fiber characterized by a high density and extensibility and a sticking temperature of above 185° C., comprising a copolymer of 65 to 80% by weight of acrylonitrile and 20 to 35% by weight of an alkyl  $\alpha$ -acylamino acrylate wherein the acyl group is the unsubstituted acyl group of a saturated aliphatic monocarboxylic acid containing 2 to 4 carbon atoms and the alkyl group contains 1 to 4 carbon atoms.

2. A synthetic fiber characterized by a high density and extensibility and a sticking temperature of 185° C. to 210° C., comprising a copolymer of 65 to 80% by weight of acrylonitrile and 20 to 35% by weight of methyl  $\alpha$ -acetaminoacrylate.

3. A synthetic fiber characterized by a high density and extensibility and a sticking temperature of 185° C. to 210° C. comprising a copolymer of 65 to 80% by weight of acrylonitrile and 20 to 35% by weight of ethyl  $\alpha$ -acetaminoacrylate.

References Cited in the file of this patent

UNITED STATES PATENTS

|    |           |               |               |
|----|-----------|---------------|---------------|
| 15 | 2,404,722 | Houtz         | July 23, 1946 |
|    | 2,461,383 | Isaacs et al. | Feb. 8, 1949  |
|    | 2,527,863 | Webb          | Oct. 31, 1950 |
| 10 | 2,570,200 | Bruson        | Oct. 9, 1951  |